

Feb. 17, 1959

A. M. PETRENKO

2,874,075

METHOD OF WATERPROOFING PAPER, CLOTH OR FUR  
AND PRODUCTS PRODUCED THEREBY

Filed Oct. 3, 1956

FIG. 1.



FIG. 2.



FIG. 3.



INVENTOR  
ALEXANDER M. PETRENKO

BY *Holcombe Hetherill & Brubbs*  
ATTORNEYS

# United States Patent Office

2,874,075

Patented Feb. 17, 1959

1

2,874,075

## METHOD OF WATERPROOFING PAPER, CLOTH OR FUR AND PRODUCTS PRODUCED THEREBY

Alexander M. Petrenko, Paris, France, assignor to Petren Products Inc., York, Pa., a corporation of Delaware

Application October 3, 1956, Serial No. 613,600

8 Claims. (Cl. 117—140)

This invention relates to a process for the preparation of a liquid which when applied will render paper and paper products, cloth, leather, wood, jute and jute products waterproof. Also applied to furs and fabrics, it makes the same waterproof and acts additionally as a protection against moths and similar insects.

Heretofore water repellent papers have been prepared by applying many types of sizings, one of which is known as "Aquapel" and consists in sizing the paper with an alkylketene dimer. Various other types of sizings using clay, starch, alum and other agents have been extensively used. All of these processes coat the surface of the paper web so as to improve the surface texture thereof and form a barrier over the fiber web that is more or less resistant to water. None of these processes impart a degree of water repellency to the cellulose fiber itself. All of the prior processes treat the surface of the web and not the fiber, which goes to constitute the web.

It is an object of the process of this invention to produce a waterproof paper.

It is also an object of this invention to impregnate the fibers of the paper with a material that will impart to the fibers themselves a water repellency, and thereby produce a waterproof product.

It is also an object of this invention to produce a process that will treat cloth, leather, wood and jute to render the same waterproof.

A further object of this invention is to provide a treatment for furs and wool materials that will render the same waterproof and repellent to moths and other insects.

The various features of novelty which characterize this invention are pointed out with particularity in the claims annexed to and forming part of this specification. For a better understanding of the special objects obtained by its use, reference should be had to the specification and examples therein in which is illustrated and described the preferred embodiment of this invention.

Fig. 1 is a flow sheet showing the preparation of the two solutions, the mixing of the solutions, the separation of the precipitated lead sulphate and the application of the final solution to paper web, cloth or fur.

Fig. 2 is an enlarged view of a cloth impregnated with the solution.

Fig. 3 is a sectional view on line 3—3 of Fig. 2 and shows the impregnation within the fiber of the cloth.

Briefly, this invention comprises the preparation of a solution, the components of which are critical, and the application of this solution to the fiber web during the process of manufacture of paper, or to the paper after it has been manufactured.

Two solutions are prepared; one, a solution of lead acetate is prepared by dissolving 48 grams of lead acetate in 500 cc. of water at normal room temperature in the neighborhood of 70° F. to 80° F. A second solution is prepared by dissolving 32 grams of potassium alum (neutral) in 500 cc. of water. These two solutions are then mixed and allowed to stand until the precipitated lead sulphate has settled. The clear liquid is decanted and used in the following processes.

The above solution is prepared so that there are two parts of alum to three parts of lead acetate by weight. The final solution on mixing must have 80 parts of the combined chemicals to one thousand parts of water to obtain the optimum results, but may vary from 60 to 102

2

parts as explained below. It is not necessary to use C. P. chemicals as technically pure grade commercial chemicals may be employed. The lead acetate must be the neutral salt.

5 The lead acetate and the alum as pointed out above are used in the ratio of 48 grams of lead acetate to 32 grams of alum to give the optimum result. These may be varied; the lead acetate being as low as 30 grams and as high as 55 grams, and the neutral potassium alum may be as low as 30 grams and as high as 47 grams. Each dissolve in 500 cc. of water so that the final solution will be in the neighborhood of one liter.

While the above proportions give the optimum results, it is possible to vary these proportions to give some degree 10 of waterproofing. For example, equal proportions of lead acetate and alum give a degree of waterproofing, but this is not comparable to the results obtained by using the three parts of lead acetate to two parts of alum.

15 The above solution is normally applied by means of a 20 perforated pipe or spray device of any type that will equally distribute the solution across the paper during its manufacture, or the paper web may be immersed in a bath of the solution. The paper must not contain an excessive amount of water at the time of the application 25 of this solution and the paper must be sufficiently dry as it leaves the last roller, so that the cutting machines will operate effectively, the drying being performed by normal means, such as by steam heated or flame heated rollers.

20 The process as set forth in this application comprises 30 the treatment of the fibers with the solution. Any sizing or other process that prevents the solution from entering the fibers through the pores thereof should be avoided.

25 While in the above application, the solution is applied 35 to the paper web during the manufacture thereof, it may also be applied to the paper after the paper has left the original manufacturing plant, in which case it is desirable that the paper be non-sized, or at most, have a small amount of sizing thereon. The usual sizings used are starch, alum, and various types of resinous material which 40 slow up absorption of the solution into the paper and therefore are objectionable when used heavily as is the usual practice.

### EXAMPLE I

45 A solution was prepared having 48 grams of lead acetate and 32 grams of alum, per liter, and the clear solution decanted from the precipitated material. This clear solution was used to waterproof kraft paper, weighing 280 grams per square meter.

50 *Running water on an inclined surface*  
KRAFT PAPER, 280 GRAMS

|                        | Waterproofed paper             |          | Ordinary paper |          |
|------------------------|--------------------------------|----------|----------------|----------|
|                        | Dry                            | Wet      | Dry            | Wet      |
| Time Necessary to Wet. | Discontinued after 31 minutes. |          | 2 minutes.     |          |
| Mullen.....            | 3.9                            | 0.8..... | 3.5            | 0.9..... |
| Rupture.....           | 1,288                          | 323..... | 1,285          | 390..... |

60 KRAFT PAPER, 224 GRAMS

|                        |                                |            |
|------------------------|--------------------------------|------------|
| Time Necessary to Wet. | Discontinued after 31 minutes. | 1 minute.  |
| Mullen.....            | 2,800                          | 0.850..... |
| Rupture.....           | 1,130                          | 340.....   |

65 IMITATION LEATHER PAPER, 280 GRAMS

|                        |                                |            |
|------------------------|--------------------------------|------------|
| Time Necessary to Wet. | Discontinued after 31 minutes. | 5 minutes. |
| Mullen.....            | 2.5                            | 0.600..... |
| Rupture.....           | 1,130                          | 300.....   |

The above test was performed in order to determine the resistance to wetting and the comparative physical properties of different types of paper after waterproofing and before waterproofing. These tests show that the different types of paper were wet within 2 minutes, 1 minute and 5 minutes respectively, while none of the samples that had been waterproofed were wet within the 31 minutes before the test was discontinued.

A second test was run on the same paper setting forth the time required for water to penetrate the waterproof paper when folded and holding 100 grams of water; and its resistance to mullen perforation after six hours and thirty minutes test:

Kraft paper, 280 grams (ordinary: non-waterproofed):  
Wet after 10 minutes test; Mullen resistance 0.800.

Kraft paper, 280 grams (waterproofed):  
Apparently not affected; Mullen resistance 1 K 650.

Kraft paper, 224 grams (ordinary: non-waterproofed):  
Wet after 10 minutes test; Mullen resistance 0.800.

Kraft paper, 224 grams (waterproofed):  
Apparently not affected; Mullen resistance 1 K 500.

Imitation leather paper, 280 grams (ordinary: non-waterproofed):  
Disintegrated to pulp after 10 minutes test.

Imitation leather paper, 280 grams (waterproofed):  
Damp after test; Mullen resistance 0 K 800.

#### EXAMPLE II

A solution was prepared having 48 grams of lead acetate and 32 grams of alum per liter, and the clear solution decanted from the precipitated material. This solution was used to waterproof a sample of military khaki clothing, measuring 1.46 meters by 1.1 meter approximately, by immersing the sample in the solution and then drying the same. This sample was tested as follows in an official laboratory:

The cloth was stretched on a wooden frame and exposed to the action of falling rain at various inclinations from 10 degrees to 70 degrees, the amount of water being approximately 2 liters per minute per square meter, and the exposure continued for a period of one week without interruption.

It was found that the unexposed surface did not present any trace of water after the test had been completed.

#### EXAMPLE III

Another test also conducted to determine the effectiveness of the waterproofing as applied above by determining the height of a column of water necessary to force the water through the cloth. Untreated samples withstood a pressure of 5 centimeters while the two treated samples withstood a pressure of 17 centimeters to 14 centimeters respectively.

Furs and natural fabrics also may be treated with this solution to render them waterproof by wetting them with the solution and then drying them. It has been found that the articles so treated are not subject to the attack of moths.

In the foregoing specification, the term "web" refers to the endless sheet of paper coming from the paper machine in its full width, or from a roll of paper in a converting operation.

The term "alum" designates the neutral double salt of aluminum sulphate and potassium sulphate and does not refer to aluminum sulphate.

There are many advantages in waterproofing the fibers of a paper web as it prevents the paper from absorbing water, losing its strength and disintegrating. This is particularly true of the straw papers and the commonly used kraft papers. The process of this invention is an inexpensive method of rendering the fibers waterproof and eliminates the necessity for sizing unless such sizing is used exclusively for increasing the strength.

Another advantage of the waterproof paper produced by this process is that a package made from a paper of

sufficient density and thickness will prevent the contents of the package from absorbing moisture.

This process has been used to waterproof cloth which will not allow the fibers to absorb water and will prevent the growth of mold spores and has been found exceptionally satisfactory for sail cloth, tents, etc.

While in accordance with the provisions of the statute there has been illustrated and described the best form of embodiment of the invention, it will be apparent to those skilled in the art that changes may be made in the process disclosed without departing from the spirit of this invention as set forth in the appended claims, and that in some cases certain features of this invention may be used to advantage without a corresponding use of other features.

What is claimed is:

1. A method of waterproofing a paper web which comprises; preparing a solution containing 32 parts of alum and 500 parts of water; preparing a second solution containing 48 parts of lead acetate and 500 parts of water; mixing these two solutions, separating the precipitate and treating said paper web with the clear solution, and drying the same.

2. A method of waterproofing the fibers of a paper web which comprises; preparing a solution containing 30 parts to 55 parts of lead acetate to 500 parts of water; preparing a second solution containing 30 parts to 47 parts of neutral potassium alum to 500 parts of water; mixing these two solutions, separating the precipitate and treating said paper web with the clear solution, and drying the same.

3. A method of waterproofing the fibers of a paper web, which comprises; preparing a solution containing 30 parts to 55 parts of lead acetate to 500 parts of water; preparing a second solution containing 30 parts to 47 parts of neutral potassium alum to 500 parts of water; mixing these two solutions, said solution before mixing having 80 parts of combined chemicals, mixing these solutions, separating the precipitate and treating said paper web with the clear solution, and drying the same.

4. A method of waterproofing natural fiber fabric which comprises; preparing a solution containing 30 to 35 parts by weight of lead acetate dissolved in water; preparing a second solution containing 30 to 37 parts by weight of neutral potassium alum dissolved in a further quantity of water to make a total of approximately 1000 parts by weight of water when mixed; mixing these two solutions, separating the precipitate and treating said fabric with the clear solution, and drying the same.

5. A method of treating furs and natural fabrics to render them waterproof and moth repellent, which comprises; preparing a solution containing 30 to 35 parts by weight of lead acetate dissolved in water; preparing a second solution containing 30 to 37 parts by weight of neutral potassium alum dissolved in a further quantity of water to make a total of approximately 1000 parts by weight of water when mixed; mixing these two solutions, separating the precipitate and impregnating the material and drying the same.

6. A waterproof fibrous material having within the pores of the fibers a soluble reactant product of two parts neutral potassium alum and three parts lead acetate.

7. A method of treating a felt product to render the same waterproof and moth repellent, which comprises; preparing a solution containing 30 to 35 parts by weight of lead acetate dissolved in water; preparing a second solution containing 30 to 37 parts by weight of neutral potassium alum dissolved in a further quantity of water to make a total of approximately 1000 parts by weight of water when mixed; mixing these two solutions, separating the precipitate and impregnating the material and drying the same.

8. A method of waterproofing a paper web; preparing a solution comprising dissolving between 30 and 47 parts by weight of alum in water, dissolving between 30 and

55 parts by weight of lead acetate in a further quantity of water, mixing the two solutions, adding water to make approximately 1,000 parts total weight of water, separating the precipitate and treating said paper web with the clear solution and drying the same.

References Cited in the file of this patent

UNITED STATES PATENTS

644,250 Kipling et al. Feb. 27, 1900

|             |                   |                |
|-------------|-------------------|----------------|
| 690,868     | Menzies           | Jan. 7, 1902   |
| 2,189,564   | Goldhammer        | Feb. 6, 1940   |
| 2,236,074   | Schwartz          | Mar. 25, 1941  |
| 2,271,492   | Bryce             | Jan. 27, 1942  |
| 5 2,391,620 | Quarles et al.    | Dec. 25, 1945  |
| 2,653,902   | Thurmon           | Sept. 29, 1953 |
| 2,790,736   | McLaughlin et al. | Apr. 30, 1957  |